# EUROPEAN PATENT SPECIFICATION

(11) **EP 1 656 460 B1**
(45) Date of publication and mention of the grant of the patent: **01.04.2009**
(21) Application number: 03817975.0
(22) Date of filing: 12.08.2003
(51) Int. Cl.: C14C 3/20, C14C 3/22

(54) **A PROCESS FOR THE PREPARATION OF A SYNTHETIC TANNING AGENT**
VERFAHREN ZUR HERSTELLUNG EINES SYNTHETISCHEN GERBSTOFFS
PROCEDE DE PREPARATION D'UN AGENT DE TANNAGE SYNTHETIQUE

(43) Date of publication of application: 17.05.2006
(73) Proprietor: Council of Scientific and Industrial Research, New Delhi 110 001 (IN)
(72) Inventor: KANTHIMATHI, Mookandi, Adyar, Chennai 600 020 (IN); THANIKAIVELAN, Palanisamy, Adyar, Chennai 600 020 (IN); RAO, Jonnalagadda, Adyar, Chennai 600 020 (IN); NAIR, Balachandran, Unni, Adyar, Chennai 600 020 (IN); RAMASAMI, Thirumalachari, Adyar, Chennai 600 020 (IN)
(74) Representative: Srinivasan, Ravi Chandran
(86) International application number: PCT/IB2003/003592
(87) International publication number: WO 2005/014865

(56) References cited:
- EP-A- 0 428 481
- WO-A-94/26789
- US-A- 5 340 365
- THANIKAIVELAN P ET AL: "A NOVEL FORMALDEHYDE-FREE SYNTHETIC CHROME TANNING AGENT FOR PICKLE-LESS CHROME TANNING: COMPARATIVE STUDY ON SYNTAN VERSUS MODIFIED BASIC CHROMIUM SULFATE" JOURNAL OF THE SOCIETY OF LEATHER TECHNOLOGIES AND CHEMISTS, NORTHAMPTON, GB, vol. 97, 2002, pages 127-136, XP009012586 cited in the application

## Description

### Technical Filed

The present invention relates to a process for the preparation of a synthetic tanning agent. More particularly the present invention provides a process for the preparation of a organo-polymeric substance, which is free from formaldehyde, using for tanning leather. This polymeric substance has enormous potential application as pretanning as well as retanning agent in leather processing industry.

### Background Art

Synthetic tanning agents are conventionally prepared by the condensation of naphthalene/phenol sulphonic acid or urea with formaldehyde as reported by Sharphouse (Leather Technicians Handbook, Vernon Lock Ltd., London, 1983).

As reported by Stille and Campbell (High Polymer, 27, 14, 1972), the phenolformaldehyde condensed product, which is essentially a low molecular weight resinous material, has always a possibility of eliminating unreacted phenol or formaldehyde, thereby posing a risk of adding to toxicity.

Denzinger et al (U.S. Patent 5,425,784, 1995) have prepared water-soluble graft polymers of monosaccharides, oligosaccharides, polysaccharides and derivatives with crotonic acid, maleic acid, maleic anhydride, fumaric acid, citraconic acid, citraconic anhydride, C₁ -C₈-alkyl- and hydroxyalkyl esters of acrylic acid, methacrylic acid or crotonic acid, mono- and di- C₁ -C₈ -alkyl and -hydroxyalkyl esters of maleic acid, fumaric acid and citraconic acid, acrylamide, methacrylamide, methacrolein, acrylamido-methylpropanesulfonic acid, N-vinylimidazole and mixtures, and used as a tanning agent for the self-tanning, pretanning, simultaneous tanning and retanning of pelts and skins. But these polymers do not produce leathers having fine grain, good fullness, affordable heat stability and uniform colour.

Wehling et al (U.S. Patent 5,340,365, 1994) have used naphthalene sulphonic acid condensate in the production of chrome leathers. They have reported that this condensation product can be used for pretreatment of delimed and bated pelts. Even though the properties of the chrome tanned leathers do not differ from those of conventionally chrome tanned, the condensed product was prepared using formaldehyde, which on ageing may undergo photo oxidation and release formaldehyde which may pose occupational hazards (Suspected carcinogens: A sub life of the National Institute for Occupational Safety and Health (NIOSH) substances list, 2nd ed. Washington DC: US Dept of Health, Education and Welfare NIOSH,1976.). Moreover the developed chrome 5 tanning method is associated with release of chromium in the effluent beyond the stipulated limit (2 ppm as Cr) as reported by Buljan (World Leather, November, 65, 1996).

Thus it is observed that even though the phenols and phenolic acid resins based on formaldehyde condensation have exhibited freedom of choice with respect to degree of 10 cross linking, molecular weight, particle size etc, the main limitations of using these polymeric condensates are the following.
a) They considerably lighten the color and when the amount used is too large, it will lead to a rubber-like handle of the leather.
b) The tanned leathers undergo photo oxidation due to the presence of active methylene bridge.
c) Slow release of formaldehyde from the tanned leathers on ageing may pose hazardous environment.

Current chrome tanning method poses severe problems due to its associated environmental problems. Industry has taken great pains to improve the chromium exhaustion. Prentiss and Sigafoos (Journal of American Leather Chemists Association, 70, 481, 1975) have reported that the use of poly acrylic and poly methacrylic acids in chrome tanning improves the chrome exhaustion. Lakshminarayana et al (Journal of the American Leather Chemists Association, 85, 425, 1990) recommends an acrylic acid based syntan as retanning agent for chrome tanned leathers, which is prepared by the graft copolymerization of acrylic ester and methacrylic acid onto a mixture of sulfated fish oil and alginic acid using free radical polymerization. But the major limitation associated with this product is that it leads to poor light fastness and heat resistance. Moreover, the acrylic syntans, which are generally attached to the protein through weak linkage, result in either low exhaustion in processing bath or more leaching out during subsequent wet operations. Christner et al (U.S. patent No 4,961,750, 1990) have reported the preparation of thio containing chromium poly acrylate tanning agents by complexing the chromium ion and an acrylate polymer together with a heterocycle containing nitrogen, oxygen, or sulfur atom, having a molecular weight between 200 and 30,000, which can be offered to prickled skins or hides. The main disadvantage in this tanning agent is the slow release of oxides of sulphur, which is carcinogenic.

The above limitations have prompted the researchers to explore possibilities of incorporating metal ion onto a polymeric matrix to form a complex for using as tanning salt. Keeping in mind the toxic hazards caused by formaldehyde, attempts have been made to prepare synthetic tanning agent, which is free from formaldehyde, as reported by Suresh et al (Journal of Cleaner Production, 9, 483, 2001) and Thanikaivelan et al (Journal of American Leather Chemists Association, 97, 127, 2002), who have also demonstrated the use of a synthetic tanning agent based on complexation of chromium with acrylic polymer and sulfonated aromatic condensates in the presence of organic ligands for self-tanning of delimed pelts and retanning applications. The use of this product result in improved exhaustion of chromium when applied on delimed pelts and hence reduces the total dissolved solids in the effluent. The major limiting feature here is that the preparation of the syntan involves employing chromium salt for complexation, thereby giving rise to the problem of toxicity associated with chrome.

### Objects of the invention

The main objective of the present invention is to provide a process for the preparation of a synthetic tanning agent, which obviates the drawbacks as detailed above.

Another objective of the present invention is to prepare a chromium exhaust aid, which can be offered to delimed pelts along with commercial BCS thus avoiding pickling process thereby reducing the total dissolved solids in the effluent.

Still another objective of the present invention is to prepare a formaldehyde free polymeric network, which helps in preventing the precipitation of chromium at lower pH values.

Yet another objective of the present invention is to prepare a polymeric product, which can be used as a retanning agent and provides leathers with improved fullness, grain firmness with uniform dyeing.

### Description of the invention

Accordingly, the present invention provides a process for the preparation of synthetic organo-polymeric tanning agent free from formaldehyde used for tanning leather, said process comprising the steps of:
(a) reacting an aromatic compound with sulfuric acid at temperature in the range of 40 to 60°C to obtain sulfonized aromatic compound;
(b) adding one or more organic ligands to the sulfonized aromatic compound obtained in step (a) and heating the mixture at temperature in the range of 60 to 80° C; 10
(c) adding one or more multi-functional polymers to the mixture of step (b) and heating the same at temperature in the range of 40 to 100° C to obtain a reaction mixture;
(d) adding water to the reaction mixture of step (c) and adjusting the pH value of the same in the range of 3.0 to 3.5;and
(e) optionally, aerating the reaction mixture and drying the reaction mixture of step (d) to obtain the synthetic organo-polymeric tanning agent.

In an embodiment of the present invention wherein in step (a), the aromatic compound 20 used contains 1-14 carbon atoms.

In another embodiment of the present invention wherein in step (a), the aromatic compound is reacted with sulfuric acid for a time period in the range of 50 to 250 minutes.

In yet another embodiment of the present invention wherein in step (a), 1 to 5 moles of sulfuric acid is used per mole of aromatic compound.

In still another embodiment of the present invention wherein in step (a), the aromatic compound used is selected from the group consisting of naphthene, anthracene, or phenol.

In one more embodiment of the present invention wherein in step (b), the organic ligand used is selected from the group consisting of formic acid, citric acid, phthalic acid, salicylic acid, oxalic acid or their sodium salts ether individually or in combination.

In one another embodiment of the present invention wherein in step (b), 0.01 to 0. mole of organic ligand is used per mole of the aromatic compound.

In a further embodiment of the present invention wherein in step (c), the multi-functional polymer is selected from the group consisting of polyacrylic acid, methacrylic acid or mixture thereof.

In an embodiment of the present invention wherein in step (c), 0.001 to 0.01 mole of multi-functional polymer is used per mole of the aromatic compound.

In another embodiment of the present invention wherein in step (d), 5 to 25 moles of 10 water per mole of aromatic compound is added to the reaction mixture.

In yet another embodiment of the present invention wherein in step (d), the pH of the reaction mixture is adjusted by adding sodium bicarbonate or by sodium hydroxide solution.

In still another embodiment of the present invention wherein in step (e), the reaction mixture is aerated by passing air /inert gas through the same.

In one more embodiment of the present invention wherein in step (e), the reaction mixture is aerated for the time period in the range of 30 to 60 minute.

In one another embodiment of the present invention wherein in step (e), the reaction mixture is dried either by drum drying or by spray drying.

In a further embodiment of the present invention wherein in step (e), the reaction mixture is dried at temperature in the range of 130 to 260°C.

In a further more embodiment of the present invention wherein the synthetic organo-polymeric tanning agent thus obtained has chromium exhaust in the range of 90 to 99 %.

The process of the present invention is described below in detail.

An aromatic compound having up to 14 carbon atoms is sulfonated by known method using 1 - 5 moles sulfuric acid per mole of aromatic compound for a period of not less than 90 min at a temperature in the range of 40 - 160°C. The temperature of the reaction mass is then adjusted in the range of 60 - 80°C and an aqueous mixture of 0.01 - 0.1 mole of organic ligand per mole of aromatic compound is added to the said mass. 0.0001 - 0.01 mole of multi functional polymer per mole of aromatic compound is then added to the said reaction mixture. Heating is allowed to continue for a period not less than 60 minutes at a temperature in the range of 60 - 80°C, pH of the resulting mixture is then adjusted at a range of 3.0 - 3.5 by known method to obtain the synthetic tanning agent in slurry form.

The above slurry is subjected, as optional step, to aeration for a period of 30-60 minutes followed by conventional drying at a temperature in the range of 130 - 260°C to obtain the synthetic tanning agent in powder form.

The novelty and non-obviousness of the present invention lies in polymerizing the multi functional polymer with sulfonated aromatic compound, pretreated with organic ligand, thereby forming an organo-polymeric matrix, free from formaldehyde, having potential application in leather industry for not only ensuring an eco-friendly approach in chrome tanning by way of eliminating the conventional pickling process and the resulting problem of total dissolved solids (TDS) associated with the effluent, but also suggesting an exhaust aid for chrome because of its multiple carboxyl groups, thereby ensuring an economical eco-benign approach for leather tanning.

The invention is described in detail in the following examples, which are provided by way of illustrations only and therefore should not be construed to limit the scope of the present invention.

### Example 1

500 gms of naphthalene and 771 ml of concentrated sulfuric acid were taken into a 2 litre round bottom flask fitted with a stirrer. The contents of the flask were heated for 180 minutes at 40°C with constant stirring. A drop of the resulting mass was taken in a beaker and 2 ml of water was added to the beaker with shaking. A clear solution, without free naphthalene smell was obtained. This confirms the completion of sulfonation. The sulfonated mass was transferred to a reactor fitted with a thermometer, stirrer and a dropping funnel. The mass was stirred continuously for a period of 10 min while maintaining the temperature at 60°C. A mixture of 14 gms sodium citrate, 17 gms phthalic acid, 11 gms sodium formate in 70 ml of water was added to the above sulfonated mass and stirring was continued at 60°C.

40 gms of polyacrylic acid was added to the sujphonic acid mixture and the mixture was heated to 80°C for 1 hour. A small portion of the reaction mixture was taken in a beaker and 2 ml water was added to the mass. The pH of the solution in the beaker was adjusted to 3.5 and a clear solution was obtained indicating the completion of the reaction. About 1400 ml of water was added to the mass and transferred to a bucket after cooling the reaction mass to room temperature. The pH of the mass was raised to 3.5 by adding a solution of 140 gms of sodium hydroxide in 350 ml water, followed by the addition of an aqueous solution of 350gms of sodium bicarbonate in 700 ml water. The slurry was filtered using a cloth of pore size 5-10u. The filtrate was drum dried at 130°C and the white powder was stored in a plastic container.

The product was offered to delimed goatskins at an offer of 1.5% along with 5% BCS at a float of 20%. The drum was run for 1 hr and 80% water was added. Running was continued for another hr and the penetration was assessed by checking uniform blue color along the cut section. The pH of the solution and the cut section was found to be 4.2. The bath was drained and the wet blue leathers were piled. Next day the leathers were post tanned using a conventional upper leather-processing recipe. The chromium exhaustion of the spent tan liquor was found to be 94%. The fullness of the crust leathers was found to be superior to that of conventional chrome tanned leathers.

### Example 2

534 gms of anthracene and 326 ml of concentrated sulfuric acid were taken in a 2 litre round bottom flask fitted with a stirrer. The contents of the flask were heated to 140°C for 90 minutes with continuous stirring, ml of the mass was taken in a beaker and 3 ml water was added with shaking. It was observed to forma clear solution without free naphthalene smell, confirming the completion of sulfonation. The sulfonated mass was transferred to a reactor fitted with a thermometer, stirrer and a dropping funnel. The mass was stirred continuously for a period of 10 min. while maintaining the temperature at 80°C. A mixture of 5.4 gms oxalic acid, 4.14 gms salicylic acid and 10 gms phthalic acid dissolved in 50 ml water was added to the above sulfonated mass and stirring was continued at 80°C.

1.5 gms of poly methacrylic acid was added to the sulphonic acid mixture and the mixture was heated to 80°C for 1 hour. A small portion of the reaction mixture was taken in a beaker and 2 ml water was added to the mass. The pH of the solution in the beaker was adjusted to 3 and a clear solution was obtained indicating the completion of the 30 reaction. About 540 ml of water was added to the mass and transferred to a bucket after cooling the reaction mass to room temperature. The pH of the mass was raised to 3 by adding a solution of 220 gms of sodium hydroxide in 500ml water, followed by the addition of an aqueous solution of 200 gms of sodium carbonate in 400ml water. The slurry was aerated for 45 minutes conventionally and filtered using a cloth of pore size 5-10µ. The filtrate was spray dried at 260°C and the white powder was stored in a plastic container.

The prepared syntan was added to the delimed sheepskins at an offer of 1.0% along with 5% BCS at a float of 20%. The drum was run for 1 hr and 80% water was added. Running was continued for another hr and the penetration was assessed by checking uniform blue color along the cut section. The pH of the solution and the cut section was 10 found to be 4.4. The bath was drained and the wet blue leathers were piled. Next day the leathers were post tanned using a conventional garment leather processing recipe. The chromium exhaustion of the spent tan liquor was found to be 95%. The fullness of the crust leathers was found to be superior to that of conventional chrome tanned leathers.

### Example 3

94 gms of phenol and 54 ml of concentrated sulfuric acid were taken in a 250 ml round bottom flask fitted with a stirrer. The contents of the flask were heated to 80°C for 100 minutes with continuous stirring. 1 ml of the resulting mass was taken in a beaker and 3 ml water was added. On shaking, a clear solution was obtained confirming the completion of sulfonation. The sulfonated mass was transferred to a reactor fitted with a 20 thermometer, stirrer and a dropping funnel. The mass was stirred continuously for a period of 10 min while maintaining the temperature at 80°C. A mixture of 1.1 gm citric acid, 0.28 gm salicylic acid and 0.56 gms sodium phthalate dissolved in 10 ml of water was added to the above sulfonated mass and stirring was continued at 70°C.

20 gms of polyacrylic acid was added to the sulphonic acid mixture and the mixture was heated to 70°C for 1 hour. A small portion of the reaction mixture was taken in a beaker and 2 ml water was added to the mass. The pH of the solution in the beaker was adjusted to 3.5 and a clear solution was obtained indicating the completion of the reaction. About 90 ml of water was added to the mass and, transferred to a bucket after cooling the reaction mass to room temperature. The pH of the mass was raised to 3.5 by adding a solution of 40 gms of sodium carbonate dissolved in 100 ml water, followed by the addition of a solution of 20 gms sodium bicarbonate dissolved in 50 ml water. The slurry was filtered using a cloth of pore size 5-10u. The filtrate was spray dried at 260°C and the white powder was stored in a plastic container.

The product was offered to delimed cow sides at an offer of 1.5% along with 8% BCS at a float of 20%. The drum was run for 2 hrs and 80% water was added. Running was continued for another 4 hrs and the penetration was assessed by checking uniform blue color along the cut section. The pH of the solution and the cut section was found to be 4.0. The bath was drained and the wet blue leathers were piled. Next day the leathers were post tanned using a conventional upper leather processing recipe. The chromium exhaustion of the spent tan liquor was found to be 92%. The fullness of the crust leathers was found to be superior to that of conventional chrome tanned leathers.

### Example 4

256 gms of naphthalene and 544 ml of concentrated sulfuric acid were taken in a 2 litre round bottom flask fitted with a stirrer. The contents of the flask were heated to 160°C for 90 minutes. 1 ml of the resulting m ass w as taken in a beaker and 2ml water was added to the mass with shaking. It was observed that the solution was clear indicating the completion of sulfonation. The sulfonated mass was transferred to a reactor fitted with a thermometer, stirrer and a dropping funnel. The mass was stirred continuously for a period of 10 min. while maintaining the temperature at 80°C. A mixture of 8.4 gms citric acid, 16.6 gms phthalic acid and 4 gms sodium formate dissolved in 50 ml water was added to the above sulfonated mass and stirring was continued at 80°C.

A mixture of 20 gms poly methacrylic acid and 5 gms polyacrylic acid was added to the sulphonic acid mixture and the mixture was heated to 60°C for 1 hour. A small portion of the reaction mixture was taken in a beaker and 2 ml water was added to the mass. The pH of the solution in the beaker was adjusted to 3.5 and a clear solution was obtained indicating the completion of the reaction. About 900 ml of water was added to the mass and is transferred to a bucket after cooling the reaction mass to room temperature. The pH of the mass was raised to 3.5 by adding a solution of 100 gms of sodium hydroxide dissolved in 200 ml water, followed by the addition of a solution of 300 gms sodium bicarbonate dissolved in 600 ml water. The slurry was filtered using a cloth of pore size 5-10µ. The filtrate was drum dried at 130°C and the white powder was stored in a plastic container.

The product was offered to delimed buff calfs at an offer of 1.5% along with 8% BCS at a float of 20%. The drum was run for 2 hrs and 80% water was added. Running was continued for another 4 hers and the penetration was assessed by checking uniform blue color along the cut section. The pH of the solution and the cut section was found to be 4.0. The bath was drained and the wet blue leathers were piled. Next day the leathers were post tanned using a conventional upper leather-processing recipe. The chromium exhaustion of the spent tan liquor was found to be 94%. The fullness of the crust leathers was found to be superior to that of conventional chrome tanned leathers.

The following are the advantages of the present invention:
1. The process is very simple and does not require any complicated and critical control measures.
2. Cheaper and indigenously available starting materials are used for the preparation of the polymeric syntan ensuring its cost effectiveness.
3. The process results in a polymer which is free from the hazardous elements like formaldehyde and chromium.
4. The polymeric product is freely soluble in water and hence can be offered along with basic chromium sulfate on delimed pelts.
5. The process ensures no precipitation of chromium when it is offered on delimed pelts at a pH in the range of 8 - 8.5.
6. The process ensures high uptake of chromium when compared to normal wet blue process.
7. The polymer is incorporated with aromatic sulphonic acids to impart fullness to the tanned leathers.
8. This syntan enhances the chrome up take and no release of formaldehyde in the tan liquor ensuring an eco-friendly and economically viable tanning process.
9. The product produces wet blue leathers with required fullness apart from serving as chrome exhaust aid.
10. The product can be used a co-tanning agent along with BCS and as a retanning agent.
11. The shelf life of the product is about 5-2 years.
12. The tanned leathers do not undergo photo oxidation since it does not contain any active methylene groups in the system unlike in other condensed tanning agents.

## Claims

1. A process for the preparation of a synthetic organo-polymeric tanning agent which is free from formaldehyde and is suitable for use in tanning leather, said process comprising:
(a) reacting an aromatic compound with sulfuric acid at a temperature in the range of 40 to 60°C to obtain a sulfonized aromatic compound;
(b) adding one or more organic ligands to the sulfonized aromatic compound obtained in step (a) and heating the mixture at a temperature in the range of 60 to 80°C;
(c) adding one or more multi-functional polymers to the mixture of step (b) and heating the same at a temperature in the range of 40 to 100°C to obtain a reaction mixture;
(d) adding water to the reaction mixture of step (c) and adjusting the pH value of the same in the range of 3.0 to 3.5; and
(e) optionally, aerating the reaction mixture and drying the reaction mixture of step (d) to obtain the synthetic organo-polymeric tanning agent.

2. A process as claimed in claim 1, wherein in step (a), the aromatic compound used contains up to 14 carbon atoms.

3. A process as claimed in claim 1 or 2, wherein in step (a), the aromatic compound is reacted with sulfuric acid for a time period in the range of 50 to 250 minutes.

4. A process as claimed in any one of the preceding claims, wherein in step (a), 1 to 5 moles of sulfuric acid is used per mole of aromatic compound.

5. A process as claimed in any one of the preceding claims, wherein in step (a), the aromatic compound used is selected from naphthene, anthracene, or phenol.

6. A process as claimed in any one of the preceding claims, wherein in step (b), the organic ligand used is selected from formic acid, citric acid, phthalic acid, salicylic acid, oxalic acid or their sodium salts either individually or in combination.

7. A process as claimed in any one of the preceding claims, wherein in step (b), 0.01 to 0.1 mole of organic ligand is used per mole of the aromatic compound.

8. A process as claimed in any one of the preceding claims, wherein in step (c), the multi-functional polymer is selected from polyacrylic acid, methacrylic acid and mixtures thereof.

9. A process as claimed in any one of the preceding claims, wherein in step (c), 0.001 to 0.01 mole of multi-functional polymer is used per mole of the aromatic compound.

10. A process as claimed in any one of the preceding claims, wherein in step (d), 5 to 25 moles of water per mole of aromatic compound is added to the reaction mixture.

11. A process as claimed in any one of the preceding claims, wherein in step (d), the pH of the reaction mixture is adjusted by adding sodium bicarbonate or sodium hydroxide solution.

12. A process as claimed in any one of the preceding claims, wherein in step (e), the reaction mixture is aerated by passing air/inert gas through the same.

13. A process as claimed in any one of the preceding claims, wherein in step (e), the reaction mixture is aerated for the time period in the range of 30 to 60 minutes.

14. A process as claimed in any one of the preceding claims, wherein in step (e), the reaction mixture is dried either by drum drying or by spray drying.

15. A process as claimed in any one of the preceding claims, wherein in step (e), the reaction mixture is dried at a temperature in the range of 130 to 260°C.

16. A process as claimed in any one of the preceding claims, wherein the synthetic organo-polymeric tanning agent thus obtained has chromium exhaust in the range of 90 to 99%.

17. Use of a tanning agent obtainable by a process according to any one of the preceding claims, in tanning leather.

18. A process for preparing tanned leather, which comprises:
- preparing a tanning agent by a process according to any one of claims 1 to 16; and
- tanning leather using the thus obtained tanning agent, in the presence of BCS.

## Patentansprüche

1. Verfahren zur Herstellung eines synthetischen, organo-polymeren Gerbstoffes, der frei von Formaldehyd ist und sich zur Verwendung bei der Gerbung von Leder eignet, wobei das Verfahren folgendes umfasst:
(a) das Umsetzen einer aromatischen Verbindung mit Schwefelsäure bei einer Temperatur im Bereich von 40 bis 60 °C unter Bildung einer sulfonierten, aromatischen Verbindung;
(b) das Zugeben von einem oder mehreren organischen Liganden zu der in Stufe (a) erhaltenen sulfonierten, aromatischen Verbindung und das Erwärmen des Gemisches auf eine Temperatur im Bereich von 60 bis 80 °C;
(c) das Zugeben von einem oder mehreren multifunktionellen Polymeren zu dem Gemisch von Stufe (b) und das Erwärmen des Gemisches auf eine Temperatur im Bereich von 40 bis 100 °C unter Bildung eines Reaktionsgemisches;
(d) das Zugeben von Wasser zum Reaktionsgemisch von Stufe (c) und das Einstellen des pH-Werts des Gemisches auf den Bereich von 3,0 bis 3,5; und
(e) gegebenenfalls das Belüften des Reaktionsgemisches und das Trocknen des Reaktionsgemisches von Stufe (d) unter Bildung des synthetischen, organo-polymeren Gerbstoffes.

2. Verfahren nach Anspruch 1, wobei in Stufe (a) die verwendete aromatische Verbindung bis zu 14 Kohlenstoffatome enthält.

3. Verfahren nach Anspruch 1 oder 2, wobei in Stufe (a) die aromatische Verbindung mit Schwefelsäure für eine Zeitspanne im Bereich von 50 bis 250 Minuten umgesetzt wird.

4. Verfahren nach einem der vorstehenden Ansprüche, wobei in Stufe (a) 1 bis 5 mol Schwefelsäure pro 1 mol der aromatischen Verbindung verwendet werden.

5. Verfahren nach einem der vorstehenden Ansprüche, wobei in Stufe (a) die verwendete aromatische Verbindung aus Naphthen, Anthracen oder Phenol ausgewählt wird.

6. Verfahren nach einem der vorstehenden Ansprüche, wobei in Stufe (b) der verwendete organische Ligand aus Ameisensäure, Citronensäure, Phthalsäure, Salicylsäure, Oxalsäure oder deren Natriumsalzen entweder einzeln oder in Kombination ausgewählt wird.

7. Verfahren nach einem der vorstehenden Ansprüche, wobei in Stufe (b) 0,01 bis 0,1 mol des organischen Liganden pro 1 mol der aromatischen Verbindung verwendet wird.

8. Verfahren nach einem der vorstehenden Ansprüche, wobei in Stufe (c) das multifunktionelle Polymere aus Polyacrylsäure, Methacrylsäure und Gemischen davon ausgewählt wird.

9. Verfahren nach einem der vorstehenden Ansprüche, wobei in Stufe (c) 0,001 bis 0,01 mol des multifunktionellen Polymeren pro 1 mol der aromatischen Verbindung verwendet wird.

10. Verfahren nach einem der vorstehenden Ansprüche, wobei in Stufe (d) 5 bis 25 mol Wasser pro 1 mol der aromatischen Verbindung zum Reaktionsgemisch gegeben werden.

11. Verfahren nach einem der vorstehenden Ansprüche, wobei in Stufe (d) der pH-Wert des Reaktionsgemisches eingestellt wird, indem man eine Natriumbicarbonat- oder Natriumhydroxidlösung zugibt.

12. Verfahren nach einem der vorstehenden Ansprüche, wobei in Stufe (e) das Reaktionsgemisch belüftet wird, indem man Luft/Inertgas durch das Gemisch leitet.

13. Verfahren nach einem der vorstehenden Ansprüche, wobei in Stufe (e) das Reaktionsgemisch für eine Zeitspanne im Bereich von 30 bis 60 Minuten belüftet wird.

14. Verfahren nach einem der vorstehenden Ansprüche, wobei in Stufe (e) das Reaktionsgemisch durch Trommeltrocknung oder Sprühtrocknung getrocknet wird.

15. Verfahren nach einem der vorstehenden Ansprüche, wobei in Stufe (e) das Reaktionsgemisch bei einer Temperatur im Bereich von 130 bis 260 °C getrocknet wird.

16. Verfahren nach einem der vorstehenden Ansprüche, wobei der auf diese Weise erhaltene synthetische, organo-polymere Gerbstoff eine Chromerschöpfung (chromium exhaust) im Bereich von 90 bis 99 % aufweist.

17. Verwendung eines Gerbstoffes, der nach dem Verfahren eines der vorstehenden Ansprüche erhältlich ist, beim Gerben von Leder.

18. Verfahren zur Herstellung von gegerbtem Leder, umfassend:
- das Herstellen eines Gerbstoffes durch ein Verfahren nach einem der Ansprüche 1 bis 16; und
- das Gerben von Leder unter Verwendung des auf diese Weise erhaltenen Gerbstoffes in Gegenwart von BCS.

## Revendications

1. Procédé pour la préparation d'un agent de tannage organopolymère et synthétique qui est exempt de formaldéhyde et qui est utilisable pour le tannage de cuir, ledit procédé comprenant :
(a) la réaction d'un composé aromatique avec de l'acide sulfonique à une température dans l'intervalle de 40 à 60°C pour obtenir un composé aromatique sulfoné ;
(b) l'addition d'un ou plusieurs ligands organiques au composé aromatique sulfoné obtenu dans l'étape (a) et le chauffage du mélange à une température dans l'intervalle de 60 à 80°C ;
(c) l'addition d'un ou plusieurs polymères multifonctionnels au mélange de l'étape (b) et le chauffage de ceux-ci à une température dans l'intervalle de 40 à 100°C pour obtenir un mélange réactionnel ;
(d) l'addition d'eau au mélange réactionnel de l'étape (c) et l'ajustement de la valeur du pH de celui-ci dans l'intervalle de 3,0 à 3,5 ; et
(e) l'aération facultative du mélange réactionnel et le séchage du mélange réactionnel de l'étape (d) pour obtenir l'agent de tannage organopolymère synthétique.

2. Procédé selon la revendication 1, dans lequel dans l'étape (a), le composé aromatique utilisé contient jusqu'à 14 atomes de carbone.

3. Procédé selon la revendication 1 ou 2, dans lequel dans l'étape (a), le composé aromatique réagit avec de l'acide sulfurique sur une durée dans l'intervalle de 50 à 250 min.

4. Procédé selon l'une quelconque des revendications précédentes, dans lequel dans l'étape (a), de 1 à 5 mol d'acide sulfurique sont utilisées par mole de composé aromatique.

5. Procédé selon l'une quelconque des revendications précédentes, dans lequel dans l'étape (a), le composé aromatique utilisé est choisi parmi le naphtène, l'anthracène ou le phénol.

6. Procédé selon l'une quelconque des revendications précédentes, dans lequel dans l'étape (b), le ligand organique utilisé est choisi parmi l'acide formique, l'acide citrique, l'acide phtalique, l'acide salicylique, l'acide oxalique ou leurs sels de sodium soit individuellement, soit en combinaison.

7. Procédé selon l'une quelconque des revendications précédentes, dans lequel dans l'étape (b), de 0,01 à 0,1 mol de ligand organique est utilisée par mole du composé aromatique.

8. Procédé selon l'une quelconque des revendications précédentes, dans lequel dans l'étape (c), le polymère multifonctionnel est choisi parmi le poly(acide acrylique), l'acide méthacrylique et des mélanges de ceux-ci.

9. Procédé selon l'une quelconque des revendications précédentes, dans lequel dans l'étape (c), de 0,001 à 0,01 mol de polymère multifonctionnel est utilisée par mole du composé aromatique.

10. Procédé selon l'une quelconque des revendications précédentes, dans lequel dans l'étape (d), de 5 à 25 mol d'eau par mole du composé aromatique sont ajoutées au mélange réactionnel.

11. Procédé selon l'une quelconque des revendications précédentes, dans lequel dans l'étape (d), le pH du mélange réactionnel est ajusté par addition d'une solution de bicarbonate de sodium ou d'hydroxyde de sodium.

12. Procédé selon l'une quelconque des revendications précédentes, dans lequel dans l'étape (e), le mélange réactionnel est aéré en faisant passer de l'air/un gaz inerte à travers celui-ci.

13. Procédé selon l'une quelconque des revendications précédentes, dans lequel dans l'étape (e), le mélange réactionnel est aéré sur une durée dans l'intervalle de 30 à 60 minutes.

14. Procédé selon l'une quelconque des revendications précédentes, dans lequel dans l'étape (e), le mélange réactionnel est séché soit par séchage en tambour, soit par séchage par pulvérisation.

15. Procédé selon l'une quelconque des revendications précédentes, dans lequel dans l'étape (e), le mélange réactionnel est séché à une température dans l'intervalle de 130 à 260°C.

16. Procédé selon l'une quelconque des revendications précédentes, dans lequel l'agent de tannage organopolymère synthétique ainsi obtenu présente une libération de chrome dans l'intervalle de 90 à 99 %.

17. Utilisation d'un agent de tannage pouvant être obtenu par un procédé selon l'une quelconque des revendications précédentes dans le tannage de cuir.

18. Procédé pour la préparation de cuir tanné, lequel comprend :
- la préparation d'un agent de tannage par un procédé selon l'une quelconque des revendications 1 à 16 ; et
- le tannage de cuir utilisant l'agent de tannage ainsi obtenu en présence de BCS.
